

1

3,585,051

METHOD OF POLISHING SURFACES  
Keith Liddell Johnson, Matteson, Ill., assignor to  
Swift & Company, Chicago, Ill.  
No Drawing. Filed Dec. 8, 1966, Ser. No. 600,051  
Int. Cl. C08h; C09d; C09g

U.S. Cl. 106—3

8 Claims

## ABSTRACT OF THE DISCLOSURE

An improved method for polishing a surface in the course of an aqueous washing operation is set forth. The method comprises dispersing in at least one of wash and rinse water a fatty imidazoline salt of a strong monoprotic acid to form a dispersion and merely contacting the surface with the dispersion to produce a lustrous, water repellent polish thereon.

The present invention relates to new and improved preparations for polishing surfaces and a method therefor. More particularly, it relates to a method for imparting a water repellent polish to a surface by contacting said surface with a solution of a self-polishing fatty imidazoline salt.

The use of wash-wax and wax-rinse self-waxing formulations in automobile washing establishments such as the familiar car washing establishments and the newer coin operated self service variety has grown rapidly in recent times. These formulations containing certain cationic surfactants provide an improved appearance on automobile surfaces. They also reduce labor requirements because the beading effect of the cationic surfactant component of the formulations enables the pressure blower system at the exit of the automatic car wash to blow a greater portion of residual rinse water from an automobile.

Prior self-waxing formulations have been blends of various surfactants, kerosene, silicone oils, waxes and other similar materials which achieve the desired effect. Illustrative of such formulations are those disclosed in U.S. Pat. 3,222,213. While performing adequately these formulations have certain inherent disadvantages which have been unsolved heretofore and have caused considerable expense to car washing establishment operators. One disadvantage encountered when these formulations are utilized is that they deposit a greasy or waxy film on the glass surfaces of an automobile that must be wiped from these areas. For example, if this film is not wiped off the windshield of a car, there will be considerable smearing upon subsequent operation of the windshield wipers. Another disadvantage encountered with some of these formulations is the necessity of having to buff the treated surface in order to bring out the desired luster. Additionally, the amount of formulation to be used per car to achieve the desired results is appreciable, being in the range of from about 2 to about 10 ounces per car. Thus, as a result of this high use level, the operating costs are significantly increased.

It is, therefore, a principal object of the present invention to provide an improved method for polishing surfaces, particularly automobile surfaces, utilizing a self-polishing composition which does not deposit a greasy or waxy film on the surface.

Another object of the invention is to provide an improved method for polishing surfaces, particularly automobile surfaces, in a more economical manner than has been possible heretofore.

A further object is to provide an improved method for applying a lustrous shine to a surface without necessitating buffing the surface.

Other objects will be apparent to one skilled in the art from the following detailed description of the invention.

2

Generally, the present invention comprises contacting a surface, particularly an automobile surface, with a solution of a strong monoprotic acid salt of a fatty imidazoline. These fatty imidazoline salts may be represented by the following structural formula:



wherein R is an alkenyl group containing from 11 to 23 carbon atoms, R' is a lower alkyl group and X<sup>—</sup> is an anion of a strong monoprotic acid. In a preferred embodiment of the invention, R is an unsaturated hydrocarbon containing from 11 to 23 carbon atoms and an average of from about 0.5 to about 2.0 groups of unsaturation per chain.

20 The preparation of these fatty imidazoline salts is described in the literature and is readily carried out by reacting a mono substituted ethylene diamine and a fatty unsaturated acylating material containing from 12 to 24 carbon atoms in the acyl group and preferably containing an average of from about 0.5 to about 2.0 groups of unsaturation per chain. The resulting reaction product is then put in contact with a strong monoprotic acid to form a salt.

25 Examples of suitable fatty unsaturated acylating compositions which can be employed as reactants include 30 vegetable oils or the fatty acids derived therefrom such as soybean oil, cotton-seed oil, sesame oil, safflower oil, tall oil, olive oil, and the like; marine oils such as menhaden oil, cod liver oil, whale oil and the like; and any animal base sources of unsaturated fat. These materials 35 can be reacted either as the triglyceride with or without subsequent removal of glycerin, or as their alkyl esters or as their fatty acids.

40 Suitable substituted ethylene diamine reactants include 45 amino ethyl ethanolamine, diethylene triamine, mono-methyl ethylene diamine, monoethyl ethylene diamine and, generally, N-alkyl ethylene diamines wherein the alkyl group contains up to about 10 carbon atoms and is either unsubstituted or substituted with non-reactive substituents such as methyl, ethyl, propyl, butyl, hydroxyl 45 benzyl groups and the like.

50 It has been discovered that for the fatty imidazoline reaction products to perform adequately in the method of the present invention, it is necessary to form a salt of the fatty imidazolines with a strong monoprotic acid. Suitable monoprotic acids which may be employed include such acids as hydrochloric, hydrobromic, sulfamic, nitric and like acids. Salts of weak acids such as acetic, formic, citric, lactic and the like and salts of polyprotic acids such as sulfuric, phosphoric, tartaric and the like are not suitable.

55 The fatty imidazoline salts of strong monoprotic acids are generally gels or even crystalline solids. However, for these compositions to be useful in the method of the 60 present invention, they must be in solution. Therefore it is necessary to dissolve the imidazoline salts in a suitable solvent. It has been found that it is desirable to employ a glycol ether type solvent for this purpose, although other solvents commonly referred to as coupling agents or 65 hydrotopes such as ethyl alcohol, n-propyl alcohol, isopropyl alcohol and the like may also be used. Exemplary of suitable glycol ether type solvents are ethylene glycol monobutyl ether, diethylene glycol monobutyl ether, butoxy ethoxy propanol, dipropylene glycol monomethyl ether and the like.

70 The fatty imidazoline salt solutions may be used in the method of the present invention to impart a lustrous, water repellent polish to a surface. These compositions

## 3

may be administered to the surface either as a formulated component of the washing detergent or as a post-washing, pre-rinse additive. The use of these compositions has the advantage of extremely low use concentrations. A further advantage of these compositions is that they achieve the desired polishing results without requiring any admixture with waxy materials. As a result, they do not deposit a waxy or greasy film on the surface and, therefore, do not necessitate an additional wiping step after processing.

When intended for use as a rinse additive, the fatty imidazoline salt compositions are prepared in aqueous solution. The amount of said solution to be used to polish a given surface will depend on such factors as the size of the surface to be polished, the concentration of the solution being used and like factors. When the compositions are used in the rinse water to polish an automobile surface, it has been found that best results are achieved by dispersing an amount of fatty imidazoline salt in the range of from about  $\frac{1}{16}$  ounce to about  $\frac{1}{4}$  ounce in a sufficient quantity of rinse water to rinse an automobile. The quantity of water utilized to rinse an automobile is generally in the range of from about 5 to about 10 gallons of water. In a preferred embodiment of the invention, about  $\frac{1}{8}$  ounce of fatty imidazoline salt is introduced into from about 5 to about 10 gallons of rinse water.

A procedure for preparing an aqueous solution of a fatty imidazoline salt for use in an aqueous automobile washing operation as a component of the rinse water is as follows. The producer may prepare an aqueous solution of a fatty imidazoline salt at a concentration of from about 5 to about 30% based on the weight of the water by dissolving it in a suitable solvent such as the above mentioned glycol ether type solvents. This stock solution is then shipped to the user. The stock solution is diluted by the user to give a feed solution. This feed solution should be dilute enough to make it practical to meter the solution into the rinse water in a manner such that from about  $\frac{1}{16}$  ounce to about  $\frac{1}{4}$  ounce of fatty imidazoline salt is dispersed in the rinse water utilized to rinse each car, generally from about 5 to about 10 gallons of water (from about .00625 ounce to about .05 ounce fatty imidazoline salt per gallon of water).

The fatty imidazoline salt compositions when intended for use as a component of the washing detergent will provide a highly lustrous finish to the clean surface. The compositions lend themselves to formulation with foam boosters such as the alkylolamine derivatives of coconut oil and sequestering agents such as tetra-sodium ethylene diamine tetra acetate in a detergent formulation. The amount of composition to be used is variable within a broad range, but the dispersion of an amount of fatty imidazoline salt from about 0.5 to about 3.0 ounces per gallon of wash water has been found to provide especially good results.

The following examples are set forth for the purpose of illustration only and are not to be construed as limiting the present invention in any respect.

## EXAMPLE I

A stock solution was prepared containing  $\frac{3}{4}$  gallon of a solution of the hydrochloride salt of 1-(2-hydroxy ethyl)-2-heptadecenyl imidazoline dispersed in  $4\frac{1}{4}$  gallons of water (15% concentration). Subsequently, the stock solution was diluted at a rate of 5 gallons of stock solution per 50 gallons of water (1½% concentration) in order to prepare a feed solution. This feed solution was then utilized in the rinse section of an automatic car washing establishment. Approximately, 8 ounces of the feed solution were metered into the rinse water (from 5 to 10 gallons of water) utilized to rinse each car processed. It was found that the automobile surfaces so treated exhibited lustrous, water repellent shines as well as improved water beading characteristics.

## 4

## EXAMPLE II

Tall oil fatty acids (280 parts) were reacted with N-methylethylenediamine (74 parts) for 2 hours under 2 atmospheres pressure at  $130^{\circ}$  C. The vessel was then vented and contents were heated to  $200^{\circ}$  C. and the water evolved was distilled out of the reaction mass. The temperature was held at  $200^{\circ}$  C. for an additional 2 hours and 30 minutes. The resulting product was cooled to room temperature and dispersed in water at a concentration of 5% and neutralized with a dilute solution of sulfamic acid to a pH of 6. The resulting solution was found to impart a lustrous, water repellent finish to an automotive acrylic lacquer finish when 5 ounces of the solution which had been dispersed in 5 gallons of rinse water was sprayed on a clean automobile surface.

## EXAMPLE III

Soybean oil (285 parts) was reacted with diethylenetriamine (103 parts) at an absolute pressure of 20 centimeters of mercury and a temperature of  $145^{\circ}$  C. for 2 hours. Then the temperature of the reaction mass was raised to  $185^{\circ}$  C. and the pressure was lowered to a value of 15 millimeters absolute. The reaction mass was then cooled and diluted to a concentration of 50% with isopropyl alcohol. This 50% solution of material was treated with a 2% solution of nitric acid until the pH of the solution had raised to a value of 5.73. When 125 ounces of the resulting solution were metered into 6 gallons of rinse water in the rinse section of an automatic car wash, the dispersion imparted a lustrous shine to an automobile surface.

## EXAMPLE IV

Menhaden oil (295 parts) was heated to  $200^{\circ}$  C. after which N-aminoethylethanolamine (104 parts) was added over a 15 minute period. The resulting product was dissolved in 500 parts of dipropylene glycol monomethyl ether and then neutralized with hydrochloric acid so that the pH of a 5% aqueous solution of this concentrate was 5.47. This material was then blended with equal parts by weight of 1.8 to 1 equivalent ratio condensate of diethanolamine with coconut oil. The resulting product provided excellent polishing characteristics when 40 ounces of the 5% aqueous solution were dispersed per gallon of wash water in a car washing formulation.

## EXAMPLE V

Tall oil fatty acids (500 parts) were heated to  $120^{\circ}$  C. At this temperature diethylenetriamine (167 parts) was added while the temperature of the reaction mass continued to rise to a value of  $137^{\circ}$  C. Approximately 32 milliliters of material were removed by distillation from the reaction mass while the pressure in the system remained at 10 centimeters of mercury. Two hours later the temperature of the reaction mass was raised to  $195^{\circ}$  C. and an additional 50 milliliters of material were removed. The resulting product was then molecularly distilled at a pressure of 232 microns and a temperature of  $230^{\circ}$  C. The resulting distillate was cooled and dispersed in water at a 5% concentration and neutralized to a pH of 6.81 with dilute hydrochloric acid. When 20 ounces of the 5% aqueous solution were dispersed per gallon of wash water, an excellent polish was imparted to the washed automobile surface.

## EXAMPLE VI

Soybean oil (1000 parts) and N-aminoethylethanolamine (317 parts) were blended together to form an emulsion and this emulsion was heated in a sealed agitated autoclave to a temperature of  $427^{\circ}$  F. for a period of 2 hours. After this period, the reaction mass was cooled and neutralized with a 10% solution of sulfamic acid. The resultant material was a thick pasty mass. When this product was dispersed in water (85.05 grams (3 ounces) per gallon of water), it provided an excellent shine to an automobile surface when used as a post-washing, pre-rinse additive.

5

Obviously many modifications and variations of the invention may be made without departing from the spirit and scope thereof, and therefore, only those limitations should be imposed as are indicated in the appended claims.

I claim:

1. An improved method for polishing an automobile surface during an aqueous washing and rinsing operation, said method comprising: dispersing in the rinse water a fatty imidazoline salt, in an amount of from about .00625 ounce to about .05 ounce per gallon of water, said salt having the general formula



wherein R is an alkenyl group containing from 11 to 23 carbon atoms, R' is a lower alkyl group, and X<sup>-</sup> is an anion of a strong monoprotic acid selected from the group consisting of hydrochloric, hydrobromic, sulfamic, nitric, and mixtures thereof; and thereafter contacting said automobile surface with the aqueous dispersion of fatty imidazoline salt.

2. The method of claim 1 wherein R is an unsaturated hydrocarbon containing an average of from about 0.5 to about 2.0 groups of unsaturation per alkenyl groups.

3. The method of claim 1 wherein the fatty imidazoline salt is the salt of 1-(2-hydroxy ethyl)-2-heptadecenyl imidazoline.

4. The method of claim 1 wherein the fatty imidazoline salt in an amount of from about  $\frac{1}{16}$  ounce to about  $\frac{1}{4}$  ounce is dispersed in from about 5 to about 10 gallons of rinse water.

5. The method of claim 1 wherein the fatty imidazoline salt in an amount of about  $\frac{1}{8}$  ounce is dispersed in from about 5 to about 10 gallons of rinse water.

6. An improved method for polishing an automobile surface during an aqueous washing operation, said method

6

comprising: dispersing in the wash water a fatty imidazoline salt, in an amount of from about 0.5 ounce to about 3.0 ounces per gallon of wash water, said salt having the general formula



10 wherein R is an alkenyl group containing from 11 to 23 carbon atoms, R' is a lower alkyl group, and X<sup>-</sup> is an anion of a strong monoprotic acid selected from the group consisting of hydrochloric, hydrobromic, sulfamic, nitric, and 15 mixtures thereof; and thereafter contacting said automobile surface with the aqueous dispersion of fatty imidazoline salt.

7. The method of claim 6 wherein R is an unsaturated hydrocarbon containing an average of from about 0.5 to 20 about 2.0 groups of unsaturation per alkenyl group.

8. The method of claim 6 wherein the fatty imidazoline salt is the acid salt of 1-(2-hydroxy ethyl)-2-heptadecenyl imidazoline.

## References Cited

UNITED STATES PATENTS

|           |         |                       |          |
|-----------|---------|-----------------------|----------|
| 2,466,517 | 4/1949  | Blair et al. -----    | 21—2.7X  |
| 2,468,163 | 4/1949  | Blair et al. -----    | 21—2.7X  |
| 3,086,870 | 4/1963  | Sheldahl et al. ----- | 106—10   |
| 3,086,871 | 4/1963  | Sheldahl et al. ----- | 106—10X  |
| 3,222,201 | 12/1965 | Boyle et al. -----    | 252—152X |

JULIUS FROME, Primary Examiner

JOAN B. EVANS, Assistant Examiner

U.S. Cl. X.R.

106—14; 117—127; 134—29; 148—6.4; 252—152, 390